

Feb. 12, 1957

H. A. WILHELM ET AL  
ELECTRODEPOSITION OF URANIUM

2,781,304

Filed Aug. 15, 1946

Fig. 1



Fig. 2



Inventors:

Harley A. Wilhelm  
Donald H. Ahmann

By: Robert A. Lassonde  
Attorney.



nium from a fused bath containing uranium halide and in the presence of uranium carbide.

2. The process which comprises electrodepositing uranium from a fused bath containing uranium halide and an alkaline earth metal halide in the presence of uranium carbide.

3. The process which comprises electrodepositing uranium from a fused bath containing uranium halide and an alkali metal halide in the presence of uranium carbide.

4. A continuous process for electrodepositing uranium which comprises conducting the electrolysis from a bath containing a uranium halide and sodium chloride in the presence of uranium carbide.

5. A process of forming a uranium salt which comprises subjecting uranium carbide to anodic treatment in a fused light metal halide bath.

6. A continuous process for electrodepositing uranium which comprises conducting the electrolysis from a bath containing uranium tetrafluoride in the presence of uranium carbide.

5 7. A continuous process for electrodepositing uranium, which comprises subjecting an electrolysis bath containing a uranium halide and a halide of light metal maintained between 500° and 800° C. to a voltage of 1-30 volts and a current density of 0.1-5 amperes/cm.<sup>2</sup> in the presence of uranium carbide.

10 15 References Cited in the file of this patent  
Van Liempt, Z. fur Elektrochem., vol. 31, pp. 249 and 250 (1925).  
Driggs et al.: Ind. & Eng. Chem., vol. 22, pp. 516 and 517, (1930).